

Oct. 6, 1953

J. A. PHINNEY

2,654,698

## LAW-TEMPERATURE DISTILLATION OF COAL.

Filed May 3, 1950



## UNITED STATES PATENT OFFICE

2,654,698

LOW-TEMPERATURE DISTILLATION  
OF COALJohn A. Phinney, Mount Lebanon, Pa., assignor  
to Pittsburgh Consolidation Coal Company,  
Pittsburgh, Pa., a corporation of Pennsylvania

Application May 3, 1950, Serial No. 159,727

7 Claims. (Cl. 202—9)

1

This invention relates to the distillation of coal and, more particularly, to the low temperature distillation of coal to yield tar, a high B. t. u. gas, and solid product or char composed of particles having a substantially uniform volatile matter content.

It has previously been proposed to distill coal at low temperatures by contacting the coal in finely divided form with sufficient hot solid distillation residue from previously distilled coal to heat the fresh coal to its distillation temperature. In such distillation systems, the solid product is a mixture comprising carbonaceous distillation residue which has been subjected only to the average temperature of the distillation zone and carbonaceous distillation residue which has been heated to a temperature substantially higher than the average temperature in the distillation zone. Thus, the total solid product is a mixture of two carbonaceous distillation residues having different volatile matter content. Since the product char represents a major proportion of the total distillation yield, it is imperative that this product possess properties rendering it suitable for use in one or more industrial applications. Generally, the most important industrial application is that of fuel for power plants. In such plants, it is highly desirable that the fuel have a uniform volatile matter content which is as high as possible, preferably in the neighborhood of 10% or higher. Unfortunately, the volatile matter content of the solid product mixture obtained by previous systems of this type is non-uniform and generally is less than 10%.

Accordingly, the primary object of this invention is to provide a process of distilling coal at low temperatures which will yield in addition to tar and high B. t. u. gas a solid char product composed of particles having substantially the same volatile matter content which is at least 10%.

In accordance with the present invention, finely divided fresh coal and preheated finely divided carbonaceous distillation residue from previously distilled coal are fed to a distillation zone. The temperature of the preheated distillation residue is sufficiently high to raise the temperature of the fresh coal to the point where it distills. The size consistencies of the fresh coal and of the preheated distillation residue are sufficiently different to permit the ready separation of the preheated distillation residue from the distillation residue produced from the fresh coal in the distillation zone. The two streams of differently sized solids are thoroughly mixed in the distilla-

2

tion zone to permit the transfer of heat from the preheated residue to the fresh coal whereby distillation of the latter is effected. The volatile products including tar and gas are separately recovered from the mixture of solid products. The latter mixture, consisting of particles of two different size consistencies, is conducted to a separation zone and there separated by any suitable means, such as elutriation into its two differently sized components. The freshly produced distillation residue is then discharged as product while the preheated residue is recycled to a combustion zone where at least a portion of the carbon content is oxidized to elevate the temperature of the residue to the desired level. It is then recycled to the distillation zone to repeat the operation.

Since the carbon content of the recycled residue is continuously being depleted in the combustion zone, it is necessary from time to time to discharge a portion thereof in the form of ash or low volatile residue, and replenish the residue from previously distilled coal of substantially the same size consistency. The latter may be accomplished by crushing a portion of the freshly produced distillation residue to the desired size and feeding it to the system or by circulating a predetermined amount of finely divided fresh coal of the same size consistency as the recycled residue. The distillation of this latter coal will provide the necessary residue to replace that discharged. Or, if more convenient, the recycled distillation residue may be replenished from an outside source of previously distilled coal.

In the preferred embodiment of my invention the recycled distillation residue has a size consistency sufficiently smaller than that of the fresh coal fed to the distillation zone to permit its ready separation from the solid distillation of the fresh coal by elutriation. In such an embodiment, the gas used to elutriate the differently sized particles may serve to carry the finer sized recycled residue to the combustion zone. Furthermore, flue gas from the combustion zone can be employed as the elutriation gas, thus providing a self-sufficient system.

The practice of my invention as briefly outlined above preserves all the advantage of distilling coal by direct contact with hot distillation residue and at the same time yields a char product composed of particles, all of which have substantially the same volatile content. This content is also substantially higher than that otherwise possible. For example, instead of a volatile matter content of 8% for the char produced without separation of the different distillation residues, a vol-

atile matter content of 15% or more may be obtained by the practice of this invention under otherwise similar conditions. Such an improvement increases considerably the value of the char as a fuel for power plants and the like.

For a better understanding of my invention, reference is had to the following detailed description and drawing in which is shown diagrammatically a preferred embodiment of my invention.

The apparatus which I prefer to employ for the practice of my invention and its operation will now be described. Numeral 10 designates a horizontal cylindrical retort mounted for rotation about its longitudinal axis. This retort and its mode of operation is more fully described in the copending application of C. E. Lesher, Serial Number 11,964, filed February 28, 1948. Finely divided fresh coal of a predetermined size consistency is fed into a retort 10 from a storage 15 hopper 12 through a conduit 14. Concurrently therewith, preheated distillation residue from previously distilled coal is fed into the same retort through a conduit 16. The size consistency of this preheated residue is sufficiently smaller 20 than that of the fresh coal to permit its ready separation by elutriation from the distillation residue of the fresh coal, as will be more fully described later. The retort is rotated to effect mixing of the two types of solids to permit transfer of heat from one to the other. The temperature of the preheated residue is sufficiently high to insure that the average temperature reached in the retort is the distillation temperature of the coal. In general, the temperature 25 of the distillation zone lies in the range of 850° to 1050° F.

The volatile products, including gas, tar and the mixture of solid products, are discharged from the retort into a separation zone 18. Here 40 the volatile products are led through a cyclone separator 20 to a discharge conduit 22. The gas and tar may subsequently be separated in conventional fashion. The solids in the separation zone 18 and also those recovered in the cyclone separator 20 are conducted through conduits 24 and 26, respectively, to an elutriator 28. Elutriation gas is introduced in the elutriator at the bottom thereof through a conduit 30. The velocity of this gas is so regulated as to effect separation of the two differently sized particles forming the mixture of solids content therein in a manner well known in the art. The larger sized particles consisting substantially entirely of fresh distillation residue from the coal feed of the retort is discharged from the bottom of the elutriator as high volatile matter product char through conduit 32.

The finer sized particles consisting of the preheated residue and any fresh distillation residue that may have been reduced to the size of the preheated residue is conveyed by the elutriation gas through a conduit 34 to a combustor 36. This combustor comprises a vertical elongated vessel comprising a lower section 38 of substantially cylindrical conformation and a higher section 40 likewise of substantially cylindrical conformation but of greater diameter than the lower section. The solids are introduced into the lower section 38 where they form a bed through which air or other oxidizing gas is circulated from a feed conduit 42. The velocity of the air is regulated to effect fluidization of the solids in the combustor. The solids are oxidized sufficiently to raise the temperature of the mass of solids

to that desired. This temperature is substantially higher than the average temperature prevailing in the distillation retort 10. Its exact value will depend upon the temperature desired in the distillation zone and upon the quantity of residue recycled. The products of combustion or flue gas are removed from the combustor through a cyclone separator 44 to a discharge conduit 46. Solids removed from this gas in the cyclone separator are returned to the bed through dip-leg 48. The hot distillation residue is discharged into conduit 16 for readmission to the distillation retort to repeat the above cycle.

A portion of the flue gas from discharge conduit 46 may be employed as the elutriation gas for the elutriator 28. In this case, the conduit 30 is connected to conduit 46 with a suitable valve arrangement (not shown) being provided to regulate the quantity of gas required. A pump 50 is disposed in the line 30 to develop the necessary pressure and circulation rate. The conduit 30 may likewise be arranged in heat exchange relation with the inlet air conduit 42 to make use of the heat content of the flue gas for preheating the air.

The recycling of the finer sized distillation residue through the combustion zone results in a depletion of the carbon content of the solids. This depletion may be carried to the point where substantially all of the carbon on the residue is oxidized to produce the necessary heat of distillation, but not necessarily. A certain amount of this depleted residue is discharged from the system through conduit 52. Replenishment of this discharge material may be accomplished in a number of different ways. Preferably, a predetermined amount of fresh coal fines having a size consistency corresponding to that of the recycled residue is introduced into conduit 14, which carries the main portion of the coal, from a storage hopper 54 through conduit 56. These coal fines are distilled in retort 10 and discharged therefrom as distillation residue having a size substantially the same as that of the preheated residue fed to the retort. These fines are added to the recycled material by the elutriation of the solid products in the elutriator 28. Another procedure is to crush a portion of the high volatile product char removed from the discharge conduit 32 through a conduit 58 to a crusher 60. This crusher effects reduction of the particle size sufficiently to convert it to the size consistency of the recycled residues. Following crushing, the fine residue is returned to the elutriator 28 through conduit 62.

In order for the above described system to operate effectively, it is necessary that the coal be distilled in the retort 10 under non-agglomerating conditions. While this presents no problem in the case of many coals, there are classes of coal which exhibit a tendency to agglomerate in the neighborhood of their distillation temperature. This agglomeration may be prevented in the manner fully described in the above mentioned copending application. The amount of recycled char is regulated so as to provide sufficient diluent to prevent the coal from agglomerating when passing through the plastic range. In the case of highly caking coals, the inert residue and fresh coal are fed separately into the rotating kiln and onto the top of a bed of char maintained at a predetermined level in the retort. In such a system the fresh coal is flash distilled so rapidly through its plastic range that no opportunity is presented for agglomeration

to take place. If it is desired to keep the amount of recycled residue at a minimum which is that required to provide the necessary heat of distillation, then any additional diluent required to aid in the prevention of agglomeration may be provided by recycling a portion of the high volatile product char from discharge conduit 32 through a conduit 64 into the same end of the rotating kiln as entered by the fresh coal and recycled residue.

As an example of the improvement obtained by the practice of the present invention, a comparison is set forth in the following table between the products produced in the system shown in the drawing without separation of the mixed solid products (case A), the recycled residue being an average portion of the total mixture, and the system embodied in the present invention (Case B). The basis of the comparison is an input of 100 pounds of green coal and a heat requirement of 770 B. t. u.'s per pound of coal to raise the temperature of the coal to 950° F. and to provide for heat loss to the atmosphere during processing. For every 100 pounds of green coal, 350 pounds of preheated distillation residue are introduced into the retort from a combustor operating at 1270° F. The coal employed is a 36% volatile matter Pittsburgh seam coal and has a size consistency of  $\frac{3}{8}$ " x 0, with about 7-10% finer than 30 mesh. The preheated residue has a size consistency of 30 mesh x 0.

Table I

|                                                     | Case A | Case B |
|-----------------------------------------------------|--------|--------|
| Carbonization Yields:                               |        |        |
| Tar, wt. percent.....                               | 15.7   | 15.7   |
| Gas, wt. percent.....                               | 6.0    | 6.0    |
| Liquor, wt. percent.....                            | 5.2    | 5.2    |
| "High Volatile Char", <sup>1</sup> wt. percent..... | 68.8   | 66.1   |
| "Low Volatile Char", <sup>1</sup> wt. percent.....  | 0.6    |        |
| To Flue Gas, wt. percent.....                       | 4.3    | 6.4    |
|                                                     | 100.0  | 100.0  |
| Analysis—"High Volatile Char": <sup>1</sup>         |        |        |
| Percent Volatile Matter.....                        | 8.1    | 14.7   |
| Percent Fixed Carbon.....                           | 77.4   | 71.8   |
| Percent Ash.....                                    | 14.5   | 13.5   |
|                                                     | 100.0  | 100.0  |
| B. t. u./lb.....                                    | 12,600 | 13,043 |

<sup>1</sup> For case A, this is a mixture of high volatile and low volatile char, while for case B it is exclusively and uniformly high volatile char.

It will be noted that the yields of char in the two cases are substantially the same yet the volatile matter content of the high volatile char in case B is 14.7% contrasted with a volatile matter of 8.1% for the mixed solid product char in case A.

According to the provisions of the patent statutes, I have explained the principle, preferred construction, and mode of operation of my invention and have illustrated and described what I now consider to represent its best embodiment. However, I desire to have it understood that, within the scope of the appended claims, the invention may be practiced otherwise than as specifically illustrated and described.

I claim:

1. In the process for low temperature distillation of coal to yield gaseous and liquid products and a solid distillation residue composed of particles having substantially the same volatile matter content, the steps comprising circulating finely divided fresh coal of a predetermined particle size consistency through a distillation zone, circulating preheated finely divided previously

distilled coal through said distillation zone in direct heat exchange relation with said fresh coal so as to form a mixture of solid products with said fresh coal, the heat required to effect distillation of said fresh coal being derived solely from said previously distilled coal, said previously distilled coal having a particle size consistency sufficiently different from that of said fresh coal to permit its ready separation from the distillation residue of said fresh coal, the total amount of distillation residue including previously distilled coal present in said distillation zone at any one time being sufficient to prevent agglomeration of said fresh coal by dilution thereof, recovering the gaseous and liquid products of distillation, separating the distillation residue of said fresh coal from said solid products, circulating at least a portion of the remaining solid products to a combustion zone where the temperature is raised by partial oxidation, recycling at least a portion of the partially oxidized solids to the distillation zone to serve as said preheated previously distilled coal, and replenishing said recycled previously distilled coal with a portion of the distillation residue.

2. In the process for low temperature distillation of coal to yield gaseous and liquid products and a solid distillation residue composed of particles having substantially the same volatile matter content, the steps comprising circulating finely divided fresh coal of a predetermined size consistency through a distillation zone, circulating preheated finely divided previously distilled coal through said distillation zone in direct heat exchange relation with said fresh coal so as to form a mixture of solid products with said fresh coal, the heat required to effect distillation of said fresh coal being derived solely from said previously distilled coal, said previously distilled coal having a particle size consistency sufficiently different from that of said fresh coal to permit its ready separation from the distillation residue of said fresh coal, circulating another but smaller amount of fresh coal of substantially the same size consistency as said previously distilled coal in direct heat exchange relation therewith, the total amount of distillation residue including previously distilled coal present in said distillation zone at any one time being sufficient to prevent agglomeration of said fresh coal by dilution thereof, recovering the gaseous and liquid products of distillation, separating the distillation residue of said first mentioned coal from said solid products, circulating the rest of the solid products to a combustion zone where their temperature is raised by partial oxidation, and returning at least a portion of the partially oxidized solids to said distillation zone to serve as said preheated previously distilled coal.

3: The process for low temperature distillation of coal in a horizontal cylindrical retort mounted for rotation about its longitudinal axis which comprises feeding into one end of said retort finely divided fresh coal and preheated finely divided previously distilled coal which is at sufficiently high temperature to raise the temperature of the fresh coal to a distillation temperature, the particle size consistency of said previously distilled coal being sufficiently smaller than that of said fresh coal to permit its ready separation by elutriation, rotating said retort whereby mixing of said fresh coal and preheated previously distilled coal is effected and distilla-

tion accomplished, the total amount of distillation residue including previously distilled coal present in said distillation zone at any one time being sufficient to prevent agglomeration of said fresh coal by dilution thereof, separately recovering the volatile and solid products, conducting said solid products to an elutriation zone, circulating gas through said elutriation zone under elutriating conditions, withdrawing the larger sized particles of freshly distilled coal from said elutriation zone, circulating the finer sized solid particles to a combustion zone, passing an oxidizing gas through said finer sized particles under fluidizing conditions, recycling at least a portion of said partially oxidized particles to said retort to serve as said preheated previously distilled coal, and replenishing said recycled solid particles by previously distilled coal of the above-mentioned size consistency.

4. In the process for low temperature distillation of coal to yield gaseous and liquid products and a solid distillation residue, the steps comprising mixing in a distillation zone fresh finely divided coal with finely divided preheated distillation residue from said coal in such proportions that the average temperature of the resulting mixture is at a distillation temperature of the fresh coal, the heat required to effect distillation of said fresh coal being derived from said preheated distillation residue, and the average particle size of said preheated residue being sufficiently smaller than that of said fresh coal to permit separation by elutriation, distilling the coal, the total amount of distillation residue including previously distilled coal present in said distillation zone at any one time being sufficient to prevent agglomeration of said fresh coal by dilution thereof, separately recovering the volatile and solid products, separating from said solid products that portion having a particle size within the range of the preheated residue fed to the distillation zone, circulating said portion to a combustion zone, partially burning said portion to raise its temperature above the average temperature in said distillation zone, and recycling this heated portion to said distillation zone to serve as said preheated residue.

5. In the process for low temperature distillation of coal to yield gaseous and liquid products and a solid distillation residue composed of particles having substantially the same volatile matter content, the steps comprising circulating finely divided fresh coal of a predetermined particle size consistency through a distillation zone, circulating preheated finely divided previously distilled coal through said distillation zone in a direct heat exchange relation with said fresh coal so as to form a mixture of solid products with said fresh coal, the heat required to effect distillation of said fresh coal being derived solely from said previously distilled coal, said previously distilled coal having a particle size consistency smaller than that of said fresh coal to permit its ready separation by elutriation from the distillation residue of said fresh coal, circulating another but smaller amount of fresh coal of substantially the same size consistency as said previously distilled coal through said distillation zone in direct heat exchange relation therewith, the total amount of distillation residue including previously distilled coal present in said distillation zone at any one time being sufficient to prevent agglomeration of said fresh coal by dilution thereof, recovering the gaseous and liquid products of distillation, conducting the

5 solid products to an elutriation zone, circulating gas through said solids in said elutriation zone under elutriating conditions, withdrawing the larger particles of distillation residue of said fresh coal from said elutriation zone, circulating the finer sized particles to a combustion zone, passing an oxidizing gas through a bed of said finer sized particles under fluidizing conditions, and returning at least a portion of these oxidized particles to said distillation zone to serve as said preheated previously distilled coal.

6. In the process for the low temperature distillation of coal to yield gaseous and liquid products and a solid distillation residue composed of particles having substantially the same volatile matter content, the steps comprising circulating finely divided fresh coal of a predetermined particle size consistency through a distillation zone, circulating preheated finely divided previously distilled coal through said distillation zone in direct heat exchange relation with said fresh coal so as to form a mixture of solid products with said fresh coal, the heat required to effect distillation of said fresh coal being derived solely from said previously distilled coal, said previously distilled coal having particle size sufficiently smaller than that of said fresh coal to permit its ready separation by elutriation from the distillation residue of said fresh coal, the total amount of distillation residue including previously distilled coal present in said distillation zone at any one time being sufficient to prevent agglomeration of said fresh coal by dilution thereof, recovering the gaseous and liquid products of distillation, conducting the solid products to an elutriation zone, circulating gas through said solids in said elutriation zone under elutriating conditions, withdrawing the larger particles of distillation residue of said fresh coal from said elutriation zone, circulating the finer sized solid particles to a combustion zone, passing an oxidizing gas through a bed of said finer sized particles under fluidizing conditions, recycling at least a portion of these oxidized particles to said distillation zone to serve as said preheated previously distilled coal, and replenishing said recycled previously distilled coal with a portion of the distillation residue.

7. In the process for low temperature distillation of coal to yield gaseous and liquid products and a solid distillation residue composed of particles having substantially the same volatile matter content, the steps comprising circulating finely divided fresh coal of a predetermined particle size consistency through a distillation zone, circulating preheated finely divided previously distilled coal through said distillation zone in direct heat exchange relation with said fresh coal so as to form a mixture of solid products with said fresh coal, the heat required to effect distillation of said fresh coal being derived solely from said previously distilled coal, said previously distilled coal having a particle size consistency sufficiently smaller than that of said fresh coal to permit its ready separation by elutriation from the distillation residue of said fresh coal, the total amount of distillation residue including previously distilled coal present in said distillation zone at any one time being sufficient to prevent agglomeration of said fresh coal by dilution thereof, recovering the gaseous and liquid products of distillation, conducting the solid products to an elutriation zone, circulating gas through said solids in said elutriation zone under elutriating conditions, withdrawing the particles of

distillation residue of said fresh coal from said elutriation zone, crushing a portion thereof to a size consistency corresponding to that of said previously distilled coal and returning it to said elutriation zone, circulating the finer sized particles from the elutriation zone to a combustion zone, passing an oxidizing gas through a bed of said finer sized particles under fluidizing conditions, and returning at least a portion of these oxidized particles to said distillation zone to serve as said preheated previously distilled coal.

JOHN A. PHINNEY.

**References Cited in the file of this patent**

**UNITED STATES PATENTS**

| Number    | Name    | Date          | Number  |
|-----------|---------|---------------|---------|
| 1,664,723 | Young   | Apr. 3, 1928  |         |
| 1,698,345 | Puening | Jan. 8, 1929  | 253,878 |
| 1,899,887 | Thiele  | Feb. 28, 1933 |         |
| 1,905,055 | Puening | Apr. 25, 1933 | 20      |

| Name            | Date          |
|-----------------|---------------|
| Hemminger       | Nov. 7, 1944  |
| Johnson         | Jan. 29, 1946 |
| Johnson         | Jan. 29, 1946 |
| Johanson        | May 13, 1947  |
| Berg            | May 11, 1948  |
| Keith           | July 20, 1948 |
| Davies et al.   | Feb. 22, 1949 |
| Sweetser et al. | Apr. 26, 1949 |
| Peck            | Aug. 30, 1949 |
| Welty Jr.       | Jan. 16, 1951 |
| Roetheli        | Dec. 18, 1951 |
| Creelman        | Aug. 5, 1952  |
| Matheson        | Oct. 14, 1952 |
| Lesher          | Dec. 16, 1952 |

**FOREIGN PATENTS**

| Country       | Date         |
|---------------|--------------|
| Great Britain | Aug. 5, 1926 |